

F. A. PARKHURST.  
MOLD AND METHOD OF CASTING.  
APPLICATION FILED APR. 2, 1919.

1,308,103.

Patented July 1, 1919.

3. SHEETS—SHEET 1.



**INVENTOR:**

FIG. 2. 26 Frederic A. Parkhurst

BY Ray S. Gehr

ATTORNEY

F. A. PARKHURST.  
MOLD AND METHOD OF CASTING.  
APPLICATION FILED APR. 2, 1919.

1,308,103.

Patented July 1, 1919.

3 SHEETS—SHEET 2.



F/G. 3.



FIG. 4.

INVENTOR:  
F. A. Parkhurst  
BY Ray S. Lehr  
ATTORNEY

1,308,103.

F. A. PARKHURST.  
MOLD AND METHOD OF CASTING.  
APPLICATION FILED APR. 2, 1919.

Patented July 1, 1919.

3 SHEETS—SHEET 3.



FIG. 5.



FIG. 8.



FIG. 6.



FIG. 9.



FIG. 7.



FIG. 10.

INVENTOR:

Frederic A. Parkhurst  
BY Ray S. Gehr  
ATTORNEY

# UNITED STATES PATENT OFFICE.

FREDERIC A. PARKHURST, OF CLEVELAND, OHIO, ASSIGNOR TO THE ALUMINUM  
CASTINGS COMPANY, OF CLEVELAND, OHIO, A CORPORATION OF OHIO.

## MOLD AND METHOD OF CASTING.

1,308,103.

Specification of Letters Patent.

Patented July 1, 1919.

Application filed April 2, 1919. Serial No. 286,970.

To all whom it may concern:

Be it known that I, FREDERIC A. PARKHURST, a citizen of the United States, residing at Cleveland, in the county of Cuyahoga and State of Ohio, have invented certain new and useful Improvements in Molds and Methods of Casting, of which the following is a specification, reference being had therein to the accompanying drawings.

- 10 This invention relates more especially to an improved form of mold gate and to an improved method of introducing molten metal into the mold cavity. While the invention, with respect to some of its features  
15 at least, is of general application, it has been developed in connection with molds for casting aluminum alloy internal combustion engine pistons and is especially applicable to the casting of cup-shaped and hollow  
20 cylindrical articles from metals or metallic alloys having relatively high crystallization shrinkages, such as characterize the aluminum alloys.

One of the objects of the invention is to  
25 avoid the formation of blow holes in the casting due to the occlusion of air or other gases.

Another object of the invention is to avoid porosity and cracks in the casting  
30 due to crystallization shrinkage.

A further object of the invention is to reduce to a minimum the bulk of the gate metal of the casting.

Other objects more or less incidental to  
35 those above stated will be apparent from the following description in which I set forth a preferred form of mold and method of casting in accordance with my invention.

In the drawings,  
40 Figure 1 is a top plan view, partially in section, of a mold having my improved form of gate.

Fig. 2 is an enlarged fragmentary vertical section on the line 2—2, Fig. 1.

45 Fig. 3 is an enlarged vertical section on the line 3—3, Fig. 1.

Fig. 4 is an enlarged fragmentary vertical section on the line 2—2, Fig. 1, with the core parts removed.

50 Fig. 5 is a horizontal section on the line 5—5, Fig. 3.

Fig. 6 is a horizontal section on the line 6—6, Fig. 3.

55 Fig. 7 is a section on the broken line 7—7, Fig. 3.

Figs. 8, 9 and 10 are fragmentary sections on the lines 8—8, 9—9 and 10—10, respectively, Fig. 3.

The construction illustrated in the drawings shows my structural improvements embodied in a permanent mold designed for the casting of aluminum alloy internal combustion engine pistons of relatively large size. Referring in detail to the construction illustrated, the mold as shown comprises a plurality of parts adapted when assembled to form a mold cavity, A, for the piston casting proper. The mold body includes a base member 1 and two complementary chambered side members 2 and 3 which are movable on the base toward and from each other and thus provide for the removal of the castings in the operation of the mold. These three main sections of the mold body are preferably formed from cast iron.

The base 1 is formed with a central depression having a cylindrical side wall 1<sup>a</sup> and a conical bottom wall 1<sup>b</sup>. Each of the side members 2 and 3 comprises an inner side wall 4, end walls 5 and 6, and top and bottom walls 7 and 8, respectively. The outer side of each of the side members is formed by a plate 9 bolted to the casting, thus closing the interior chamber 10 of the member. Handles 11, 11 are secured to the plates 9, 9 so that the side members of the mold can conveniently be moved to and from operative position on the base.

The inner side walls 4 of the complementary members of the mold body mutually engage with each other when said members are moved together as shown in Fig. 1. The wall 4 is formed between its ends with a semi-cylindrical portion 4<sup>a</sup>, and the lower parts of this semi-cylindrical wall 4<sup>a</sup> together with the cylindrical side wall 1<sup>a</sup> in the base, form the upper side wall of the casting cavity proper, the bottom of said cavity being formed by the conical bottom wall 1<sup>b</sup> of the depression in the base member. Said conical wall is formed with a central depression 1<sup>c</sup> which provides for a "work spot" on the head of the piston casting. The bottom wall of this central depression is formed by a plug 1<sup>d</sup> which is grooved on its periphery to provide vents for air and other gases.

To secure alinement of the mold members 2 and 3, in relation to each other, the base is formed with a cylindrical shoulder 12,

and coöperating cylindrical shoulders 12<sup>a</sup>, 12<sup>a</sup> are formed in each of the side members 2, 3. These coöperating shoulders 12 and 12<sup>a</sup> are struck from the same axis and thus 5 serve to effect perfect alinement of the side members in relation to each other. To insure the proper angular positioning of the side members on the base 1, the latter is provided with upstanding dowel pins 13 10 which engage semi-cylindrical recesses 13<sup>a</sup> in the side members 2, 3.

The mold is provided with a main core 14 which is preferably made of steel and is of the five part form shown in Figs. 13 to 19 15 of my U. S. Letters Patent No. 1,296,597, and is of the same general character as the core shown in the U. S. Letters Patent to Joseph H. Bamberg No. 1,296,588. For a detailed description reference may be had to 20 said Letters Patent. For the purpose of the present application it will suffice to state that the core comprises a central part 14<sup>a</sup> and two pairs of members 14<sup>b</sup>, 14<sup>c</sup> and 14<sup>d</sup>, 14<sup>e</sup> which when assembled are adapted 25 to be supported at their upper ends in the mold body so as to depend within the cavity formed therein and form the inner walls of the casting cavity proper. The main core parts are supported in the mold body by 30 engagement with a pair of liners 15, 15 which are suitably secured to the mold members 2, 3, as by screws 15<sup>a</sup>. The lower ends of the liners serve to form the annular top wall of the mold cavity. With the main core 35 parts supported in the liners 15 as shown in Fig. 2, the mold cavity takes substantially a cup shape corresponding to the trunk or skirted piston which it is desired to cast.

To insure proper angular positioning of 40 the core 14 in the mold body, the central member 14<sup>a</sup> of the core is provided with a key 16 which projects from the core and is received between wear plates 17 secured in slots in the mold members 2, 3 and their 45 liners 15, 15. Each of the core parts is provided with a suitable handle 14<sup>f</sup> to facilitate assembling of the core in the mold and its removal therefrom.

The core members 14<sup>b</sup> and 14<sup>c</sup> are shaped to 50 form a recess 14<sup>g</sup> to provide for a wrist pin boss on the casting while the members 14<sup>d</sup> and 14<sup>e</sup> are shaped to form a recess 14<sup>h</sup> for a similar purpose.

The core 14 is provided with vent passages as follows: The middle part 14<sup>a</sup> of the 55 core is formed on its opposite flat faces with longitudinal passages 14<sup>k</sup>, 14<sup>k</sup>, each of which extends from the upper end of the core part to a transverse passage 14<sup>m</sup> near the lower 60 end of the core part. Then these flat faces of the core part are formed at their lower ends with a series of vent grooves 14<sup>n</sup> extending from the bottom surface of the core upward to the transverse passage 14<sup>m</sup>, and 65 an adequate vent upward through the core

is thus provided for air and gases collecting on the bottom surface of the core. Each of the liners 15 is formed with vent grooves 15<sup>b</sup>, 15<sup>c</sup>, 15<sup>d</sup> and 15<sup>e</sup> on its bottom, inner, outer and top sides, respectively. 70

18, 18 are removable core pins slidably mounted in the mold members 2, 3 with their inner ends projecting into the boss recesses 14<sup>g</sup>, 14<sup>h</sup>. To facilitate their removal, said pins have their ends slightly tapered 75 where they engage the mold body and project into the mold cavity.

In the operation of the mold the various parts are secured in operative position by lock devices 19, 19, each of which comprises 80 a pin 19<sup>a</sup> mounted on one of the side members of the mold and a coöperating pivoted hook 19<sup>b</sup> on the other side member. When the side members 2, 3 are brought together in proper position on the base 1, the hooks 85 19<sup>b</sup> are forced down over the pins 19<sup>a</sup> so that the parts of the mold body are firmly secured together.

I turn now to a description of the gate of the mold to which my present invention more 90 particularly relates. The gate, which is formed by alining recesses in the adjacent walls 4, 4 of the mold members 2 and 3 and in the base 1, in its entirety comprises a feeder and a supply conduit. The feeder is 95 in the form of an upright cavity 20 adjacent one side of the casting cavity and extending from the bottom of the casting cavity upward to and above the upper end of said cavity, the upper part of the feeder 100 comprising a riser extension 20<sup>a</sup>. The feeder communicates with the casting cavity through a short passage 21, said passage extending, preferably, continuously from the bottom to the top of the casting cavity 105 and being relatively narrow in comparison with the greater width of the feeder cavity. The adjacent faces of the mold members 2 and 3 are formed with vent grooves 22 extending from the top of the riser chamber 110 20<sup>a</sup> to the upper surface of the mold.

The supply conduit of the gate comprises an inlet section 23 which is formed with downwardly converging walls, a lower discharge section 24 which extends from the lower end of the inlet section 23 downwardly and laterally into the bottom of the casting cavity of the mold; and an upper discharge section 25 which extends laterally from the upper end of the discharge section 24 into the upper part of the feeder 20. The discharge section 24, as well as the inlet section 23, preferably has its walls converging downwardly somewhat. At the lower end of the discharge section 24, it communicates with the bottom of the feeder 20, as well as with the casting cavity. 115 120 125

The gate parts are all formed in the side members 2, 3 of the mold, except that the lower ends of the feeder 20 and the dis- 130

charge section 24 are formed by a recess 26 in the base 1.

It is usually desirable to provide for heating the body of the metal to maintain it at a suitable temperature and I have shown burners 27, 27 mounted on brackets 28, 28, said burners being arranged so that their flames are directed through openings 9<sup>a</sup> in the plates 9, to heat the inner walls of the mold members 2 and 3, and especially the parts of the walls 4, in which the gate is formed, this arrangement insuring that the metal in the gate shall remain molten longer than that in the mold proper.

15 Preferably the surfaces of the mold, including core parts, which constitute the walls of the mold cavity are suitably coated or treated in well known manner to reduce as much as possible agitation of the 20 molten metal as it flows into contact therewith and to insure proper setting of the metal within the cavity.

My improved method of casting will readily be understood from a consideration 25 of the operation of the above described mold. The members 2 and 3 are first moved into operative position on the base 1, then the sections of the main core 14 are inserted, the locking devices 19 are driven home 30 to tightly lock the mold members 2 and 3 together and firmly clamp the main core in position. Finally the core pins 18 are introduced.

The temperatures at which the various 35 parts are maintained will depend largely upon the nature of the metal or alloy to be cast. Assuming that the burners 27 have been operated to heat the mold parts to the desired temperature, the mold is now ready 40 to receive the molten metal. Said metal is brought to the mold in any suitable manner, as by a ladle, and is poured into the inlet 23 of the gate. The marked convergence of the walls of the inlet section 23 from its upper 45 to its lower ends strongly checks the velocity of the entering metal so that it emerges from the lower end of the inlet section 23 with a reduced velocity and encounters the gently curving wall of the downwardly and laterally extending discharge section 24 smoothly and without agitation.

In the said discharge section 24 a further check on the velocity of the metal is provided both by the lateral inclination of the 55 passage and by the gradual contraction of its walls from its upper toward its lower end, so that a smooth and steady flow of metal is secured and the metal first entering the casting cavity emerges from the discharge section 24 and enters the casting cavity with little if any agitation or splashing, so as to avoid the mixing of air or gases into the metal with resultant formation of blow holes in the finished casting.

60 As the molten metal continues to flow into

the mold and its upper surface, in the casting cavity, comes into contact with the lower end of the core 14, the air above the metal either finds its way radially outward and into the annular part of the cavity in which 70 it is free to rise and escape through vent grooves 15<sup>b</sup>, 15<sup>c</sup>, 15<sup>d</sup> and 15<sup>e</sup>, formed in the liners 15, or, entering the vent grooves 14<sup>a</sup>, finds its way upward through the core to the exterior of the mold. It may be observed 75 in this connection that the venting of the air or gases overlying the relatively quiescent mass of rising metal is readily effected in the manner last described, but if there is splashing or agitation of the metal in the 80 mold, air or gas is occluded in it and I have found it practically impossible to separate such air or gas, no matter how adequate the provision for venting may be, so that a serious porosity of the casting results. This is 85 especially true of the metal first entering the mold because it seems especially difficult to separate occluded air or gas bubbles from the body of the metal which rises upward into contact with the lower end of the main 90 core. It is also particularly true in the case of castings having heavy cross sections, it being always more difficult in such cases, apparently to eliminate air or gases that become occluded in the metal. It will thus 95 be seen that the practical importance of avoiding splashing of the metal in the mold cavity is very great.

As the molten metal rises in the annular section of the mold cavity, it simultaneously 100 rises in the feeder 20, and if, at any stage of the pouring, the level of the metal rises more slowly in the mold cavity than in the feeder, the metal in the feeder will flow smoothly through the passage 21 into the 105 mold cavity and find its way in both directions around the main core to the diametrically opposite side of the cavity. As the passage 21 extends continuously from the bottom to the top of the mold cavity this smooth 110 and unagitated flow of metal from the feeder into the mold cavity can occur at any level until the cavity is entirely filled.

It is obvious that after the first entering 115 metal has filled the bottom parts of the casting cavity and the feeder, the molten metal subsequently entering beneath the surface of the bath in the cavities is bound to do so without any splashing and resultant occlusion of air or gases.

In the process of filling the casting cavity, when the level of the molten metal therein rises to the level of the second discharge passage 25, the entering metal tends to pass from the lower end of the inlet section 23 into the discharge section 25, and through it directly into the upper part of the feeder 20 and thence through the short passage 21 into the upper part of the casting cavity 125 until the latter is filled. Thereupon, by 130

reason of the hydraulic head of the metal in the inlet section of the gate, the flow continues through the discharge section 25 until the riser chamber 20<sup>a</sup> is nearly or entirely filled with the molten metal.

The metal which enters the upper part of the riser through the discharge section 25 does so at a very moderate velocity, this being insured not only by the checking of the flow in the inlet section of the gate, but also by the angular arrangement of the discharge section 25 in relation to the inlet section 23. That is to say, the very abrupt change of direction which the entering stream of metal must make when passing from the inlet section to the discharge section 25 so greatly checks its velocity that the metal is delivered into the feeder chamber quite slowly and without splashing.

20 In the filling of a mold cavity in the shape of a hollow cylinder or of a cup-shaped mold cavity such as that of the present mold, the molten metal gives up its heat to the walls of the mold and tends to freeze first at points 25 remote from the gate or source of supply and then gradually and progressively from said remote points around the main core toward the gate. It will thus be understood that it is important to maintain in the feeder section 30 of the gate a molten mass of metal upon which the metal in all parts of the mold cavity is free to draw to make up for crystallization shrinkage as the freezing progresses. In my improved form of gate the molten 35 condition of the metal in the feeder is insured by providing the separate discharge passages 24 and 25, the former entering the lower end of the feeder while the latter enters the upper part thereof. Thus there 40 is a relatively direct supply of the molten metal into the lower part of the feeder to maintain a molten supply in said lower part of the feeder to compensate for crystallization shrinkage in the lower portion of the 45 casting cavity, and also a direct supply, through passage 25 of molten metal for the upper part of the feeder so that an adequate body of molten metal is provided in the upper part of the feeder and in the riser 50 chamber to compensate for crystallization shrinkage in the upper part of the casting cavity. In other words, an adequate supply of molten metal is maintained in position to enter the casting cavity at any level to compensate for crystallization shrinkage and a 55 progressive setting of the metal in the mold is insured from points opposite the gate around the main core in both directions, then in the short passage 21 between the casting 60 cavity and the feeder and finally in the feeder itself.

After a short interval to permit the metal to set, the locking devices 19 are eased off, the core parts are withdrawn, the pins 18 65 somewhat in advance of the main core parts,

then the locking devices 19 are entirely disengaged and the mold members 2 and 3 separated to permit removal of the casting.

It will be seen that my improved method of introducing the metal into the mold cavity by means of the mold and gate structure set forth, by avoiding occlusion of air or other gases in the molten metal, prevents blow holes in the castings which would otherwise result. It will also be seen that the 70 insuring of a molten mass of metal in all parts of the feeder chamber during freezing of the metal in the adjacent parts of the casting cavity, insures a complete compensation for crystallization shrinkage in the 75 casting proper, and thereby avoids the serious porosity which would otherwise result. Furthermore, by making the gate discharge passages 24 and 25 separate from the feeder 80 cavity, I am enabled to form and dispose 85 said passages so as to insure a slow and smooth entrance of the metal into the casting and feeder cavities without expanding the feeder cavity; and therefore, since the 90 cross-sectional dimensions of the passages 90 24 and 25 can be made much smaller than those of the feeder cavity, I secure the desired result with a minimum bulk of gate metal.

I have shown my invention only in connection with molds for the production of piston castings but it is obviously applicable in the production of castings of other articles and other forms and it will be understood that the foregoing disclosure is 100 for purposes of illustration and explanation and not intended to define the scope of the invention.

What I claim is:

1. A mold having a cavity for the casting 105 proper and provided with a gate comprising an upright feeder cavity adjacent the casting cavity and communicating with the latter cavity at various levels between the bottom and top thereof through a short narrow 110 passage, an inlet passage extending downwardly and laterally and opening into the bottom of the casting cavity, and a second inlet passage extending laterally from the first inlet passage into the upper part of 115 the feeder cavity.

2. A mold having a cavity for the casting proper and provided with a gate comprising an upright feeder cavity adjacent the casting cavity and communicating with the latter cavity at various levels between the bottom and top thereof through a short narrow 120 passage, an inlet passage extending downwardly and laterally and opening at its lower end into the bottoms of the casting cavity and feeder cavity, and a second inlet 125 passage extending laterally from the first inlet passage into the upper part of the feeder cavity.

3. A mold having a cavity for the casting 130

proper and provided with a gate comprising an upright feeder cavity adjacent the casting cavity and communicating with the latter cavity at various levels between the bottom and top thereof through a short narrow passage, an inlet passage extending downwardly and laterally, said passage having downwardly converging walls and opening at its lower end into the bottom of the casting cavity, and a second inlet passage extending laterally from the first inlet passage into the upper part of the feeder cavity.

4. A mold having a cavity for the casting proper and provided with a gate comprising an upright feeder cavity adjacent the mold cavity and communicating with the mold cavity at various levels between the bottom and the top thereof through a short narrow passage, said feeder cavity being formed with a riser chamber extending above the top of the casting cavity, an inlet passage extending downwardly and laterally and opening into the bottom of the casting cavity, and a second inlet passage extending laterally from the first inlet passage into the upper part of the feeder cavity.

5. The method of introducing molten aluminum alloys or the like into a mold which consists in delivering the molten metal into the bottoms of the casting cavity and an upright feeder cavity arranged at

one side of the casting cavity, causing the metal to rise in said casting and feeder cavities from the bottoms thereof as the pouring continues, introducing molten metal into the upper part of the feeder cavity after the casting and feeder cavities have been partially filled from below to complete the filling of the same, and causing the metal to flow from the feeder cavity at various levels into the casting cavity to compensate for crystallization shrinkage.

6. The method of introducing molten aluminum alloys or the like into a mold which consists in delivering the molten metal into the bottoms of the casting cavity and an upright feeder cavity arranged at one side of the casting cavity, causing the metal to rise in said cavities from the bottoms thereof until they are partially filled, introducing molten metal into the upper part of the feeder cavity to complete the filling of the said cavities and to rise upward into a riser extension of the feeder cavity, and causing the molten metal to flow from said feeder cavity at various levels into the casting cavity to compensate for crystallization shrinkage.

In testimony whereof, I hereunto affix my signature.

FREDERIC A. PARKHURST.